

# UNITED STATES PATENT OFFICE.

JOSEPH SCHEERER, OF SAN FRANCISCO, CALIFORNIA.

## STREET-PAVEMENT AND THE METHOD OF CONSTRUCTING THE SAME.

1,195,273.

Specification of Letters Patent. Patented Aug. 22, 1916.

No Drawing.

Application filed September 15, 1913. Serial No. 789,908.

To all whom it may concern:

Be it known that I, JOSEPH SCHEERER, a citizen of the United States, and a resident of the city and county of San Francisco, State of California, have invented certain new and useful Improvements in Street-Pavements and the Method of Constructing the Same, of which the following is a specification.

10 The invention relates to street pavements employing asphalt or similar material as a binder, and particularly to the wearing or top surface of street pavements.

15 The object of the invention is to provide a street pavement which will not become smooth and slippery under service.

Another object of the invention is to provide a street pavement which possesses comparative permanency and stability.

20 A further object of the invention is to provide a method of laying a wearing surface upon other pavements.

25 The invention possesses other advantageous features which, with the foregoing, will be set forth at length in the following description where I shall outline in full that form of the invention which I have selected for description herein. The novelty of the invention will be included in the claims succeeding said description. From this it will be apparent that I do not limit myself to the showing made by said description as I may adopt many variations within the scope of my invention as set forth in said claims.

30 Asphalt and similar pavements soon become very smooth and slippery in service, due to automobile traffic and the lubricating oil dropped by the countless automobiles passing over and standing on the pavement.

40 The lubricating oil unites with the asphalt and produces a hard surface which becomes very smooth due to the travel of rubber tired wheels, producing a very dangerous pavement, even in dry weather. In wet weather, 45 the surface of the pavement becomes so slick that the driving of automobiles thereover becomes dangerous and the driving of horses impossible.

45 The pavement of my invention is of such character that it presents an even surface to traffic, but is not affected by lubricating oils and does not wear smooth and slippery, affording at all times and in all conditions of weather a perfect tractive surface. The 55 pavement of my invention, which constitutes the wearing surface, may be applied as a covering to smooth and dangerous asphalt

pavements or to macadamized, oiled, brick, granite, cement, slag, or basalt pavements.

50 My invention relates to the wearing surface of the pavement and any suitable or available foundation or base therefor may be used, although I prefer to lay it over an asphalt pavement.

55 The old pavement or base is first cleaned in a suitable manner, and when it happens to be an asphalt pavement, it is preferably, though not necessarily, heated to soften the asphalt and remove some of the lubricating oil therefrom. The pavement is then given 60 a coating, preferably a brush or spray coat of hot liquid asphaltum, which acts principally to bind the top surface to the old pavement. This asphaltum coating is then covered by a coating, preferably a brush or 65 spray coat of an asphalt compound or mixture. This mixture consists of hot liquid asphalt containing ground lime rock, plaster of Paris, pumice stone, diatomaceous earth or ground slag. It is not essential that all of 70 these materials be used in the mixture as several of those mentioned have equivalent functions. The pumice stone, diatomaceous earth and slag absorb the lubricating oil which comes up from the old pavement; the 75 plaster of Paris causes the asphalt to become stiff when cold and prevents it from flowing materially under pressure and the lime stone acts as a filler to make the mixture set harder when cool. The percentage of these 80 materials in the mixture may be varied, depending upon the base and the road conditions to be met. Over this coat I place a mineral aggregate composed principally of broken hard rock and lime stone. For this 85 purpose I prefer to use crushed basalt or granite and lime stone in the proportion of approximately fifty per cent. of each. This aggregate consists preferably of from 90 60 to 75 per cent. of rock which will pass through a 100  $\frac{3}{8}$  inch ring but will be retained by a quarter inch ring and from 25 to 40 per cent. of rock which will pass through a quarter inch ring and be retained by an eighth inch ring. This aggregate is heated and is distributed 105 over the second asphalt coat in a layer, preferably one half or three quarters of an inch thick. The aggregate is then rolled with a light hot roller. The heated rocks become embedded in the asphalt coatings which are 110 pressed upward into the interstices between the aggregate binding the same firmly together. When this surface is applied to an old asphalt pavement, some of the asphalt

of the old pavement which is softened by the heat is also forced upward between the pieces of the aggregate. The aggregate may also contain a small proportion of the oxids of 6 iron and manganese which act as a flux to bind the rock and the asphalt to produce a homogeneous mass. The asphalt enters the pores of the lime stone and forms a very firm bond therewith and the rough and 10 jagged condition of the constituent parts of the aggregate also assists in forming a tight bond. The material of the aggregate should be as free from clay as possible, since the presence of clay will produce a slippery 15 pavement. After rolling with the light roller, I apply a top dressing of about  $\frac{1}{8}$ th inch pieces of aggregate consisting of crushed hard rock such as basalt or granite, lime rock and pumice stone, which fills 20 up the larger voids on the upper surface. This is then rolled with a heavy steam roller, the roller of which is preferably heated and the increase in pressure compacts the aggregate more closely, forcing some of the asphalt 25 up and thereby binding the top dressing in place. The lime rock in the top dressing is adhered to very strongly by the asphalt producing a very stable pavement and the pumice stone is present to absorb 30 the lubricating oil which subsequently falls on the pavement. The finished pavement presents a substantially smooth, hard surface having innumerable small depressions therein, which are not removed by wear, the 35 aggregate is held very firmly together and the surface will not disintegrate.

The liquid asphalt, the asphalt mixture and the aggregate may be applied quickly and cheaply to the old pavement surface 40 from a vehicle which passes over the surface. The vehicle is provided with suitable storage compartments for the three coats or layers and is provided with suitable means for discharging the various materials onto the 45 surface. A transverse conductor having a plurality of apertures or nozzles arranged longitudinally therein is provided for the distribution of the hot liquid asphalt. Behind this conductor is a similar one for distributing the asphalt mixture on the asphalt 50 coat and behind this is a rotating screen or shuttle or other device for depositing the aggregate.

I claim:

- 55 1. In a street pavement, an asphaltic mineral structure composed of crushed hard rock, lime stone, an oil absorbing stone and an asphaltic binder.
2. In a street pavement, an asphaltic 60 mineral structure composed of crushed hard rock, lime stone, pumice stone and an asphaltic binder.
3. A street pavement comprising a rigid

foundation, a coating of asphalt on said foundation, a coating of asphalt mixture 65 consisting of asphalt, ground lime stone, ground oil absorbing stone and an asphaltic binder on said asphalt coating, and a layer of mineral aggregate of small sizes and free from clay on said asphalt mixture, the aggregate being rolled to force the asphalt upward into the interstices of the aggregate.

4. In a street pavement, a wearing surface containing crushed lime stone, pumice stone and a binder. 75

5. The method of constructing a wearing surface on a road foundation which consists in applying a coat of hot liquid asphalt, then applying a coat of a hot liquid asphalt mixture consisting of asphalt, ground lime 80 stone, ground oil absorbing stone and an asphaltic binder, then applying a layer of hot crushed mineral aggregate and then rolling the mass with a hot roller.

6. The method of constructing a wearing 85 surface on a road foundation which consists in applying a coat of hot liquid asphalt, then applying a coat of an asphalt mixture containing stiffening and oil absorbing mediums and a filler, then applying a layer of 90 hot crushed mineral aggregate, the separate pieces of which will pass through a three-eighths inch ring, then rolling the mass with a hot roller to force the asphalt upward into the interstices in the aggregate. 95

7. The method of constructing a wearing surface on a road foundation which consists in applying a coat of hot liquid asphalt, then applying a coat of hot liquid asphalt containing plaster of Paris, then applying a 100 layer of crushed mineral aggregate containing lime stone, then rolling the mass, then applying a top dressing of fine mineral aggregate containing an oil absorbing mineral and then rolling the mass with a heavy 105 roller.

8. The method of constructing a wearing surface on old asphalt pavements which consists in heating the surface of the old pavement, applying a coat of hot liquid 110 asphalt thereto, then applying a coat of hot liquid asphalt containing plaster of Paris, then applying a layer of hot mineral aggregate free from clay and containing lime stone, then rolling the mass with a hot roller, 115 then applying a top dressing of fine mineral aggregate free from clay and containing lime stone and pumice stone, and then rolling the mass with a heavy roller.

In testimony whereof, I have hereunto set 120 my hand at San Francisco, California, this 8th day of September, 1913.

JOSEPH SCHEERER.

In presence of—

H. G. PROST,

M. LE CONTE.